



US006796862B1

(12) **United States Patent**  
**Abbenhouse et al.**

(10) **Patent No.:** **US 6,796,862 B1**  
(45) **Date of Patent:** **Sep. 28, 2004**

(54) **FORKED RIB KAYAK PADDLE**

(76) Inventors: **John Abbenhouse**, 8060 - 171<sup>st</sup> Ave. NE, Redmond, WA (US) 98052; **John R. Murkowski**, 1814 N. 47<sup>th</sup> St., Seattle, WA (US) 98103

(\*) Notice: Subject to any disclaimer, the term of this patent is extended or adjusted under 35 U.S.C. 154(b) by 0 days.

(21) Appl. No.: **10/635,207**

(22) Filed: **Aug. 6, 2003**

**Related U.S. Application Data**

(60) Provisional application No. 60/401,643, filed on Aug. 6, 2002.

(51) **Int. Cl.** <sup>7</sup> **B63H 16/04**

(52) **U.S. Cl.** **440/101; 416/74**

(58) **Field of Search** **440/101; 416/70 R, 416/74**

(56) **References Cited**

**U.S. PATENT DOCUMENTS**

738,053 A \* 9/1903 Murdock ..... 416/74  
4,610,633 A \* 9/1986 Freudenberg ..... 440/101  
4,955,839 A 9/1990 Kaschper ..... 440/101  
5,820,424 A 10/1998 Steinhour ..... 440/101  
6,210,244 B1 \* 4/2001 Nordby ..... 440/101  
6,328,617 B1 \* 12/2001 Gunnell ..... 440/101  
6,568,971 B1 \* 5/2003 Abbenhouse et al. ..... 440/101  
2002/0025423 A1 2/2002 Dreher et al. ..... 423/318

**FOREIGN PATENT DOCUMENTS**

|    |         |   |         |       |         |
|----|---------|---|---------|-------|---------|
| FR | 2599331 | * | 12/1987 | ..... | 440/101 |
| GB | 1165343 |   | 9/1969  |       |         |

**OTHER PUBLICATIONS**

Machine Design, Aug. 3, 2000, "Reinforced Plastics Make Metals Look Weak" by Johnson and Greene.

\* cited by examiner

*Primary Examiner*—Stephen Avila

(57) **ABSTRACT**

A kayak paddle having at least one paddle blade is made by laying a first resin impregnated fiber preforms in a lower half of a split mold. The split mold has a bifurcated channel for producing a bifurcated rib in a back face of the paddle blade. One end of a paddle shaft is inserted into a cylindrical recess in the lower mold half, and a bifurcated foam core is inserted in the lower mold half over the bifurcated channel. A second resin-impregnated fiber preform is laid over the first fiber preform, and an upper half of the split mold is closed over the lower mold half from one end in clam-shell fashion. Heat and pressure are applied to press the molds together to create thereby a fluid wall of liquid resin which advances through the fiber preforms as the mold closes, driving air out of the fabric preforms as the resin advances through the fiber preforms, and curing the resin to produce a solid fiber-reinforced resin matrix paddle blade bonded to the paddle shaft.

**6 Claims, 11 Drawing Sheets**





Fig. 1



Fig. 1A



Fig. 1B



Fig. 2



Fig. 3



Fig. 4



Fig. 5



Fig. 6



Fig. 7



Fig. 8



Fig. 9





**FORKED RIB KAYAK PADDLE**

This is related to U.S. Provisional Application No. 60/401,643 filed on Aug. 6, 2002 and entitled "Forked Rib Kayak Paddle".

**BACKGROUND OF THE INVENTION**

This invention pertains to processes for making paddles, and more particularly to efficient processes for making superior quality kayak paddles with composite blades and the kayak paddles made by those processes.

Since the invention of the kayak by the ancient peoples of Alaska and Iceland, there has been a continual effort on the part of kayakers to improve the design and construction of kayak paddles. Efficient paddle design is an optimal balance of minimal weight, maximal strength, optimal stiffness, effective performance in the water, and low cost.

All modern high performance paddles are composite constructions of fiber reinforced resin blades on hollow shafts, also made of fiber reinforced plastic materials. The blade is normally molded in a two-part die machined to the desired blade shape, and the molded blade is then fitted to a purchased paddle shaft. Among the many problems of prior art composite paddles are excessive blade molding time because of the cure time for the resin, and excessive blade weight because of excess resin in the cured blade. The attachment of the blade to the paddle shaft is normally a lengthy, multi-step process fraught with potential for failure.

**SUMMARY OF THE INVENTION**

Accordingly, this invention provides a paddle having reduced weight and increased strength, and a fast and efficient process for making paddles with paddle blades having the desired mechanical properties of strength, light weight, durability and effective propulsion effect.

A paddle blade in accordance with this invention has a dihedral power face having a center rib extending the full length of the blade, from root to tip. On the back face of the blade, a center rib bifurcates into two branches, extending out toward the blade tip but terminating short of the blade tip. The bifurcated rib on the back face is built on a forked foam core. A groove on the back face starts at the bifurcation of the back face rib, and the center groove on the backside extends out to the blade tip between the diverging branches of the bifurcated rib. The bifurcated core produces a forked rib on the backside, straddling the dihedral center groove almost out to the tip of the paddle blade, and the power face side has a clean dihedral shape that releases the water smoothly. The forked rib on the back face increases the strength and stiffness of the blade at the usual fracture point of the blade by at least 50% while allowing a reduction of weight of as much as 20% and avoiding both paddle flutter and turbulence.

A process for making paddles in accordance with the invention includes making a two-part mold having semi-cylindrical openings for the paddle shaft so that the paddle blade may be molded and co-cured directly on the paddle shaft. The mold surfaces correspond to the ultimate outer mold line of the paddle power face and back face, and also are designed to express liquid resin from the centerline of the paddle outward toward its edges and the blade tip as the mold closes. The mold closing and heating schedule is designed to partially cure the resin so that it flows outward through the reinforcing fiber at a controlled rate, preventing resin starvation of the fiber reinforcement and ensuring complete expulsion of any air bubbles in the reinforcing

fiber. After the resin is cured, the mold is opened and the paddle is removed from the mold. The paddle edge is then trimmed by a high speed CNC router to produce a paddle that conforms exactly to the desired peripheral shape.

**DESCRIPTION OF THE DRAWINGS**

The invention and its many attendant benefits and advantages will become better understood upon reading the following detailed description of the preferred embodiments in conjunction with the following drawings, wherein:

FIG. 1 is a plan view of a paddle in accordance with this invention, showing the power face of the paddle blades;

FIGS. 1A and 1B are plan and perspective views, respectively, of the back face of the blades shown in FIG. 1, showing the forked stiffening rib;

FIG. 2 is an elevation of the paddle shown in FIG. 1;

FIG. 3 is an elevation of one paddle blade of the paddle shown in FIG. 1 and the end of the paddle shaft to which the blade is bonded;

FIG. 4 is sectional elevation on a vertical axial section plane in FIG. 3;

FIG. 5 is a schematic elevation of a press in which a matched two-part clam-shell mold is mounted for molding the paddle blades and bonding them to the paddle shaft to form the paddle shown in FIG. 1;

FIG. 6 is an elevation of the two-part mold shown in FIG. 5, illustrating the clam-shell disposition of the mold halves to each other;

FIG. 7 is a perspective view of the lower mold half shown in FIG. 6, showing the outline of the paddle blade as it will look after trimming;

FIG. 8 is a plan view of a fiber preform with a resin load used to form the paddle blade shown in FIG. 3;

FIG. 9 is a graph showing the mold closing and pressure schedule for operating the press shown in FIG. 5 to close the mold shown in FIG. 6;

FIG. 10 is a sectional end elevation of an apparatus for forming an indexing surface on the paddle shaft shown in FIG. 2; and

FIG. 11 is an enlarged sectional elevation of the paddle shaft shown in FIG. 10.

**DETAILED DESCRIPTION OF THE PREFERRED EMBODIMENTS**

Turning now to the drawings, and more particularly to FIG. 1 thereof, one end of a kayak paddle 30 in accordance with this invention is shown having a paddle shaft 32 and a paddle blade 34 at each end of the shaft 32. The shaft 32 is preferably a commercially available carbon fiber/epoxy tube purchased from any one of several suppliers of such tubes. Other shaft materials such as fiber glass/epoxy or pultruded fiberglass and carbon fiber/epoxy could be used to reduce the cost of the paddle and improve toughness, but their strength-to-weight and stiffness-to-weight ratios are generally inferior to carbon fiber/epoxy. The carbon fiber/epoxy shaft 32 has a wall thickness of about 0.055" and an outside diameter of about 1.25" which is convenient for the average man's hand, but smaller shafts, on the order of one inch, can be used for paddlers having smaller hands such as children and some women. Thicker paddle shaft wall thickness can be used to obtain greater strength, primarily of interest to recreational whitewater kayakers, but at a greater weight and cost. An indexing flat 35, shown in FIG. 2 and described in more detail below, is formed along the shaft 32 at the

position of one or both hands when gripping the paddle to assist the paddler in orienting the paddle in his hands for the optimal angle of the blade 34 with respect to the water surface. The blades 34 are made and bonded to the shaft 32 by a process described below.

The blades 34 are spoon-shaped, as shown in FIGS. 2 and 3, having a generally concave dihedral power face and a generally convex back face, with a small concave "low brace" power section 33 on the back face. A center stiffening rib 36 extends the full length of the power face of the blade 34 from root to tip, and blade fins 38 extend laterally outward from the rib 36. On the back face of the blade, shown in FIGS. 1A and 1B, a back face stiffening rib 40 has a center rib 41 that extends from the root of the paddle blade 34, where it connects to the paddle shaft 32, to an intermediate position 42 about one-quarter to one-third of the longitudinal length of the blade toward the tip 39. At the intermediate position 42, the center rib 41 splits into two branches 43 and 44, which diverge out toward the blade tip 39, but terminate short of the blade tip 39. The bifurcated or forked rib 40 on the back face is built on a forked foam core. A center groove 46 on the back face starts at the intermediate position 42 where the bifurcation of the back face rib 40 begins, and the center groove 46 on the backside extends out to the tip 39 between the diverging branches 43, 44 of the bifurcated rib 40. The two branches 43 and 44 of the forked rib 40 on the backside straddle the center groove 46 almost out to the tip 39 of the paddle blade to provide increased strength and stiffness, and the power face side has a clean dihedral shape that releases the water smoothly. The forked rib on the back face increases the strength and stiffness of the blade at the usual fracture point of the blade by 50%–100% while allowing a reduction of material and weight, and avoiding both paddle flutter and turbulence.

The blade fins 38 can be made of carbon fiber fabric/epoxy about 0.70" thick or less, or other combinations of fiber materials such as glass fiber fabric and Kevlar and carbon fiber fabric may be used to provide desired properties of strength, stiffness, toughness and light weight. The fiber materials are normally used in fiber mats, preformed to the desired thickness, length and width. Another material that has produced excellent kayak paddle blades is a thermoplastic material known as Twintex. It is fabric woven from glass fibers individually coated with a thin film of polypropylene. It does not outgas during molding, does not require curing time, and is tough and light weight, as described in greater detail below.

Another material heretofore unknown for use in kayak paddles is an aluminized fiberglass woven fabric called "Alumitex", made by Hexcell Corp. and available commercially from Composites One in Arlington, Wash. The Alumitex material is laid as the first and last ply in the fiber preform 70 described below. When using Alumitex, a clear epoxy is used as the bonding matrix to avoid obscuring the attractive silver sheen on the fabric with opaque epoxy. The primary benefit of the Alumitex material in a paddle blade, aside from its visual appeal, is the improved visibility it affords. In rescue situations involving river kayakers, it is important that object of rescue be very visible. The bright and shiny Alumitex material is very visible in a river, even in turbulent water, and facilitates locating the victim needing rescue. In addition, even in situations which are not life-threatening, it is not uncommon for a kayaker who flips in the river, fails his roll, and swims, to also lose his paddle, which floats away downstream. Typically, his paddling companions will assist in his rescue and also help retrieve his gear, including his paddle. However, paddles are often

notoriously hard to see from a kayak, but a bright shiny silver paddle is much easier to see in the water. Loss of a paddle on the river usually ends the trip for the paddler and is certainly a costly loss, so facilitating retrieval by making the paddle more visible in the water is a valuable improvement in the paddle art.

Various blade shapes and dimensions are used for various paddling environments and paddler strengths. A typical sea kayak paddle blade for an expedition sea kayaker is about 10 20.5" long and about 6.5" wide. Sea kayakers desiring more relaxed and shorter distances will usually select a narrower and sometimes longer paddle blade. Whitewater kayakers usually prefer a shorter, wider blade, e.g. 7.5" wide and 19" long. The process described herein for molding the blade can 15 easily accommodate these various blade shapes and dimensions.

The process for making the kayak paddle in accordance with this invention utilizes a two-part clam-shell mold 50 for use in a press, shown schematically in FIG. 5. The mold 50, 20 shown in more detail in FIGS. 6 and 7, includes an upper mold half 52 and a lower mold half 54. The facing surfaces of the mold halves 52 and 54 have surface contours defining the upper and lower mold lines of a mold interface 56 having the shape of the paddle blade 34. A plurality of grooves 58 25 in the lower mold half 54 define restricted flow channels 60 out of the mold interface 56 to restrict the flow of resin out of the mold during the mold closing sequence, as explained in more detail below. A semi-cylindrical axial rib channel 62 extends in the floor of the upper mold half 52 the full length 30 of the mold, and a corresponding bifurcated channel 64 extends in the mold source of the bottom mold half 54 about ⅓–⅔ of the length of the paddle mold surface, as indicated in FIG. 7, to form the axial strengthening rib 36 in the back 35 face of the paddle blade 34, as shown in FIGS. 1–4. The remaining ⅓–⅔ of the rib molding contour of the bottom mold half is reversed into a ridge to match the outer portion of the channel 62 in the upper mold half to form a U-shaped ridge 65 at the outer portion of the strengthening rib 36, as shown in FIG. 4.

40 A semi-cylindrical paddle shaft channel 66 at the paddle shaft end of the mold halves 52 and 54, as shown in FIG. 7, receives the end of a paddle shaft 32 which is supported in a V-block 67 or the like positioned along the axis of the channel 64 and the paddle shaft channel 66, and is held therein by a clamp 68. A chamfer 69 at the junction of the paddle shaft channel 66 and the axial rib channel 64 provides a smooth and attractive junction of the paddle blade 34 and paddle shaft 32 in the molded paddle 30.

45 The process of molding the paddle blade 34 and simultaneously bonding the paddle blade to the paddle shaft 32 starts with measuring two volumes of mixed liquid epoxy resin and hardener. Various resin formulations may be used, but the preferred materials are resin 833 and hardener 944 sold by Composites One in Arlington, Wash., mixed in a resin to hardener ration of 4:5. The two ingredients are preferably mixed in a resin mixer, although the ingredients can be mixed by hand if production throughput is not important.

50 The facing surfaces of the mold are coated with a mold release that is effective to prevent the epoxy formulation being used from sticking to the mold surfaces, which otherwise would present an extremely difficult clean-up job after the paddle is removed from the mold and would 55 produce a paddle with very poor surface quality. There are numerous commercial mold release products available any 60 one of them can be used that is effective. Release films are

also available and can be used, but the preferred mode is to use a spray or liquid coating material to avoid the chance of wrinkle marks produced by wrinkles in a release film.

A preselected fiber preform **70** having the desired fiber content for the paddle being made is laid on a work surface and one of the two volumes of mixed liquid epoxy resin and hardener is poured onto the fiber preform **70** in a central axial zone on the preform and is spread in a broad band **72**, as shown in FIG. 8, on the fiber preform **70** with a squeegee or the like. A cover sheet **74** of Alumitex or polybutylene terephthalate (PBT) with graphics for marketing and source identification may be laid on the lower mold half **54**, and the fiber preform **70** with its resin load is laid over the cover sheet **74** in the lower mold half **54** with the edge of the fiber preform aligned with the chamfer **69**. A molded bifurcated foam core **75** having the desired shape of the power side rib **36** and the back side bifurcated rib **40** is inserted into the end of the paddle shaft **32** and the paddle shaft is laid in the paddle shaft channel **66** and the V-block **67** with the foam core **75** lying in the axial rib channel **64**. The clamp is engaged to hold the paddle shaft **32** securely in position in the paddle shaft channel **66** over the first resin-loaded fiber preform **70**. A second preselected fiber preform **70** is laid on the work surface and the second volume of mixed resin and hardener is poured onto the second fiber preform **70** in an central axial zone, like the first. The resin is spread in a broad axial zone with a squeegee like the first, and the second resin-loaded fiber preform is laid over the end of the paddle shaft **32** and foam core **75** in alignment with the first fiber preform. A second cover sheet **74** may be laid over the second resin-loaded fiber preform **70**. The fiber preforms **70** and the cover sheets **74** are laid carefully to lie flat and avoid wrinkles which could result in an unsightly uneven appearance and could weaken the blade. To speed the production through the press, the fiber preforms can be pretensioned in a wire frame that extends beyond the molds so the workers do not need to spend time smoothing the fiber preforms to avoid wrinkles.

When the upper and lower resin-loaded fiber preforms are in place on both sides of the end of the paddle shaft **32** and the foam core **75**, the press is activated to execute and automatically timed mold closing sequence as shown in the graph in FIG. 9. The press is started at time zero and the mold halves make contact a few seconds later at point A, whereupon the pressure in the press rises almost immediately to the beginning pressure of 20 PSI at the start of the pressure ramp at point B. The pressure is gradually ramped up to the final pressure of about 45 PSI at point C over several minutes. This provides time for the resin to fully saturate the cloth as well as allowing time for air in the fabric preform **70** to be displaced from the fabric by the resin as it is driven outward and toward the paddle shaft end, as indicated by the flow arrows in FIG. 7, by the slowly closing clam-shell mold halves to the flow channels **58** and out of the paddle mold. The mold halves close in clam-shell fashion from the blade-tip end toward the paddle shaft end by virtue of the slight angle of the mold faces as indicated in FIG. 6, wherein the mold is still 0.045"-0.065" apart at the paddle shaft end when it first makes contact at the blade tip end. The upper mold half **52** can tilt slightly as necessary to execute the clam-shell closing action by virtue of the flexibility of the press which allows a small tilting motion under pressure. The temperature of the mold halves **52** and **54** is maintained constant about 170°-174° F. As the resin becomes warm in the mold, its viscosity decreases and it flows easily to wet the fabric. However, the increasing temperature accelerates the curing of the resin mixture and

its viscosity increases, thereby providing a fluid wall as it advances through the fabric preforms **70**, driving the air before it. The curing of the resin is an exothermic reaction, which raises the temperature in the mold interface to accelerate the rate of curing. At the end of the curing cycle, at point D, the pressure in the press ram is released and the mold opens, allowing the cured paddle blank to be removed.

A paddle blade **34** is now molded and bonded to the other end of the paddle shaft **32** in a similar operation to the one described above, on a similar but reversed two-part mold. Alternatively, if production through put from the molding facility is paramount, two presses could be set up parallel to and spaced apart from each other to allow workers to mold and bond the paddle blades on opposite ends of the paddle shaft **32** at the same time. Alternatively, or in addition, several sets of molds **52** and **54** could be mounted on the platens of the press, thereby increasing the production throughput from a single press.

The paddle with the molded and bonded blade blanks is mounted on a fixture which holds it securely for trimming the blade **34** to the desired profile. An efficient and accurate trimming apparatus is a CNC operated air driven router, operated at about 20,000 RPM. At that speed, the composite material is cut cleanly without shredding or chipping the epoxy material, and the CNC controller cuts the molded blade to exactly the same profile every time.

Paddle blades made of polypropylene and glass fiber do not need a cure time since polypropylene is a thermoplastic material. The preferred form of polypropylene coated glass fiber material is a co-extruded polypropylene coating on a monofilament glass fiber and provides a linear orientation of the polypropylene molecules for superior properties in the consolidated fused final product. Twintex is the commercial supplier of this material. The molding process provides heat and pressure for sufficient time to fuse and consolidate the polypropylene in the Twintex material, and then holds the formed paddle blade in the desire configuration while the polypropylene hardens enough to hold its shape. By thoroughly cleaning the end of the paddle shaft **32** and providing sufficient pressure to the Twintex material on the end of the paddle shaft, the polypropylene can be made to bond securely to the carbon fiber/epoxy material in the paddle shaft **32**.

Two fiber preforms of Twintex polypropylene/glass fiber material are prepared with the desired number of layers of the Twintex fabric and a cover sheet **74** as described previously. A clam-shell mold is preheated to about 400° F.-412° F. and the first preform is laid in the lower mold half **54**. The carbon fiber shaft **32**, with its end thoroughly cleaned of oils and mold release from its manufacture, and with the bifurcated foam core **75** protruding from the end, is set in the V-block and the paddle shaft channel **66**. The second fiber preform is laid over the first in alignment therewith, sandwiching the end of the paddle shaft **32** and the foam core **75**. The second fiber preform also has a cover sheet **74**. The molds **52** and **54** are closed and pressure of about 42 PSI is applied to the materials for about one minute or until the polypropylene is fused and the material is consolidated into a semi-solid material. The mold is then opened and the fused, bonded, formed and consolidated paddle blade blank is removed from the mold. PBT and Alumitex face skins function as a mold release as well as providing structural qualities. The hot paddle blade **34** is immediately placed in an identical mold that is at room temperature. The mold is closed and pressure of about 9-10 PSI is applied for about one minute in the cool mold while the blade **34** cools to about 170° F. or less and hardens so that it retains its shape

when removed from the cooling mold. Both forming and cooling molds can be in the same press or the forming molds can be in a separate press from the cooling molds. The paddle blade may be stiffened with a sheet of carbon fiber fabric between the face sheets and the fiber preform. If sufficient polypropylene material is available on the glass fiber, it will flow into the carbon fiber and provide a strong bond therewith. Otherwise, a small amount of epoxy resin can be used for bonding or the carbon fiber cloth can be pre-impregnated with epoxy resin in the B-stage cure condition.

An alternate process using only a single mold uses a radiant heat source to heat the polypropylene/glass fiber preforms to a temperature at which the polypropylene softens and is ready to fuse. The hot fiber preforms, with or without face sheets, are inserted into a cool mold, sandwiching the end of the paddle shaft and foam core 75, and the mold is closed with 40–50 PSI to consolidate the polypropylene and bond it to the end of the paddle shaft, as above. The mold is opened in about one minute after the blade is cool enough to retain its shape.

The polypropylene/glass paddle blade is molded to net size, so no trimming is needed except for a possible thin flash around the periphery of the paddle. The savings in labor, material cost and rapid molding rate, and the desirable properties of light weight and toughness make this material a very attractive one for kayak manufacturing.

Paddle shaft indexing flats are formed on the paddle shaft 32 in the apparatus shown in FIG. 10. A split heating mold 80 is provided with heating coils 82 connected by power and control cables to a temperature controller 84 which controls electrical power from a power source 86, such as the power grid, to the heater elements 82. The temperature in the split mold 80 is set at about 325° F. The paddle shaft 32 is inserted in the split mold 80 and a section of paddle shaft about 12 inches long is heated in the mold 80 for about 20–30 seconds, until it approaches the mold temperature and becomes soft enough to form. The heating mold 80 is opened and the hot section of paddle shaft is immediately inserted into an open split forming mold 88, and the mold is closed on the paddle shaft. One of the mold halves of the split mold 88 has an indexing surface 90 by which the soft heated paddle shaft wall is formed with the indexing surface 35. The carbon/epoxy shaft material cools quickly in the cool forming mold 88 and may be removed in 10–15 seconds. If there is a large run of paddles that are to have the indexing flats formed, the forming mold 88 may be cooled with a cooling system such as a blower 92 controlled by a blower controller 94 using a temperature transducer 95.

The profile of the indexing surface 35 on the paddle shaft 32, shown in detail in FIG. 11, includes first surface 96 that is flat or slightly curved, having a radius  $R_3$  and subtends an angle  $\phi_1$  of about 45°. On both sides of the first surface 96 are two blending surfaces 98 each having a radius of about  $R_2$  and subtending an angle  $\phi_2$  equal to about 15°. Blending surfaces 98 provide a smooth transition from the first surface 96 into the full radius surface of the paddle shaft 32. The first surface 96 lies at an angel  $\Theta$  from the plane of the power face of the fins 38 of the paddle blade 34. The angel  $\Theta$  is about 60°–85°, preferably 72°.

Obviously, numerous modifications and variations of the preferred embodiment described above are possible and will become apparent to those skilled in the art in light of this specification. Moreover, many functions and advantages are described for the preferred embodiment, but in many uses of the invention, not all of these functions and advantages

would be needed. Therefore, we contemplate the use of the invention using fewer than the complete set of noted features, process steps, benefits, functions and advantages. For example, all the process elements may be used to produce a particular part that requires the characteristics provided by each process element, or alternatively, they may be used in combinations that omit particular process elements or substitute others to give the desired characteristics of the part. Moreover, several species and embodiments of the invention are disclosed herein, but not all are specifically claimed, although all are covered by generic claims. Nevertheless, it is our intention that each and every one of these species and embodiments, and the equivalents thereof, be encompassed and protected within the scope of the following claims, and no dedication to the public is intended by virtue of the lack of claims specific to any individual species. Accordingly, it is expressly intended that all these embodiments, species, modifications and variations, and the equivalents thereof, in all their combinations, are to be considered within the spirit and scope of the invention as defined in the following claims, wherein we claim:

What is claimed is:

1. A kayak paddle having a paddle shaft and a dihedral blade with a power face on at least one end of said shaft, and a back face opposite said power face, comprising:

a center rib extending longitudinally of said power face from root to tip of said blade;

a back face rib having a center portion adjacent said blade root, and a bifurcated portion which splits into two branches, diverging out toward said blade tip and terminating short of said blade tip;

a groove on said back face, starting at the bifurcation of said back face rib, and extending out to said blade tip between said diverging branches of said bifurcated rib, producing a forked rib on said backside, straddling said center groove, and a clean dihedral shape of said power face side that releases the water smoothly;

whereby, said forked rib on said back face increases said blade strength at a usual fracture point of said blade while allowing a reduction of weight and avoiding both paddle flutter and turbulence.

2. A kayak paddle as defined in claim 1, wherein; said dihedral blade is a lay-up construction of fiber reinforced resin composite having a sheet of aluminum-coated fiberglass fabric bonded on the surface of said power face and said back face to produce a paddle blade having a bright and shiny silver appearance.

3. A kayak paddle as defined in claim 2, wherein; said fiber reinforced resin composite is made primarily of carbon fiber in a clear epoxy matrix.

4. A kayak paddle as defined in claim 2, wherein; said fiber reinforced resin composite is made primarily of glass fiber in a polypropylene matrix.

5. A process of making a kayak paddle having at least one paddle blade, comprising:

selecting two fiber preforms having resin therein;

laying one of said preforms in a lower half of a split mold, said split mold having a bifurcated channel for producing a bifurcated rib in a back face of said paddle blade; inserting an end of a paddle shaft in a cylindrical recess in said lower mold half;

inserting a bifurcated foam core over said bifurcated channel;

laying the other fiber preform over said paddle shaft end and over said first fiber preform;

**9**

closing an upper half of said split mold over said lower mold half from one end in clam-shell fashion, and applying heat and pressure to create thereby a fluid wall of liquid resin which advances through said fiber preforms as said mold closes and drives air out of said fabric preforms as said resin advances through said fiber preforms, to produce a solid fiber-reinforced resin matrix paddle blade bonded to said paddle shaft.

**10**

6. A process of making a kayak paddle as defined in claim 5, further comprising:  
laying a sheet of aluminum-coated fiberglass fabric under said one fiber preform and over said other fiber preform to produce a paddle blade having a bright and shiny silver appearance.

\* \* \* \* \*